

1

3,042,575  
METHODS OF IMPROVING THE YIELD IN ALKALINE DIGESTION OF CELLULOSIC MATERIAL  
Nils Josef Christoffer Hartler, Lidingö, Sweden, assignor to Stiftelsen Svensk Celitiosaforskning, Stockholm, Sweden, a corporation of Sweden  
No Drawing. Filed Nov. 16, 1959, Ser. No. 852,964  
Claims priority, application Sweden Nov. 24, 1958  
5 Claims. (Cl. 162—89)

The present invention relates to alkaline digestion of lignocellulosic materials, such as wood chips. The main object of the invention is to improve the yield of pulp from the digestion, but also to provide qualitative improvements of the resulting pulp, such as improved brightness and beatability. As used herein, the term "alkaline digestion" refers mainly to the sulfate and soda processes of digesting lignocellulosic materials but other methods in which digestion takes place at least partly at a pH above 7, e.g. the so-called neutral sulfite process are within the scope of the invention.

It is known from a number of published investigations that the solubility in hot alkali of a cellulosic material diminishes after it has been treated with a suitable oxidizing or reducing agent.

As a suitable oxidizing agent, sodium chloride has been mentioned (O. Samuelson and N. Hartler, Svensk Kemisk Tidskrift, 62 (1950), 197) and this result has later been confirmed and studied more closely by several researchers (A. Meller, TAPPI 34 (1951), 171, and ibid. 35 (1952), 72; H. Richtzenbain et al., Svensk Papperstidning 57 (1954), 363, and ibid. 57 (1954), 538). This oxidizing agent seems to have a selective action. The carbonyl groups of the cellulose material are oxidized to form carboxyl groups. Other oxidizing agents tested (e.g. chlorine dioxide) have little or no effect in the respect here contemplated, i.e. to reduce the hot alkali solubility in a subsequent treatment with a dilute solution of sodium hydroxide at temperatures of up to 100 to 120° C.

As a suitable reducing agent to achieve the same effect, sodium borohydride has been mentioned (A. Meller, TAPPI 36 (1953), 366, and 38 (1955), 682). In this case, too, a selective action is involved. The carbonyl groups of the cellulose material are reduced to form alcohol groups and the increased stability to alkali decreases the hot alkali solubility of the material.

In one aspect, the present invention relates to the process of adding in alkaline digestion of lignocellulosic materials, e.g. by the soda or sulfate process, a reducing agent which under the conditions prevailing in the digestion reduces carbonyl groups of cellulose, whereby the yield of pulp is enhanced and the quality of the pulp is improved in various respects.

Suitable reducing agents for this purpose are hydrides,

2

economic considerations. However, the effect of the reducing agent is not increased above a certain limit, and suitably, therefore, the amount used will be below 3% by weight of the lignocellulosic material.

The digestion is otherwise carried out by conventional methods, which need not be discussed in detail here, since they are well-known to those skilled in the art. The digestion is generally carried out at temperatures of 160–200° C. By way of example, the process of this invention can also be applied to the digestion of a lignocellulosic material which prior to digestion has been subjected to a preliminary treatment with digestion liquid of an initial pH between 1 and 11 and a temperature between 120 and 180° C.

It was also found, and this forms another aspect of this invention, that the treatment with reducing agents of the above-mentioned type can advantageously be carried out on the lignocellulosic starting material, usually wood chips. This has the advantage that carbonyl groups present in the cellulose, which form starting points for degradation of the cellulose molecule in an alkaline environment, are eliminated already before the material is contacted with the alkaline digestion liquor.

It has further been found that it is more preferable not only to carry out pretreatment with a reducing agent, but also to add a reducing agent during digestion, suitably during the period when the mixture of lignocellulosic material and digestion chemicals is brought to the desired maximum temperature, whereby also such carbonyl groups which are formed during the digestion are eliminated.

The pretreatment is suitably carried out at a temperature within the range of 0–100° C. As in the addition of reducing agent to the digestion liquor, the amount of reducing agent should suitably be at least 0.001% and preferably at least 0.01% by weight of the lignocellulosic starting material, and for economical reasons it is preferably below about 3% by weight of the lignocellulosic material.

The invention is illustrated but not limited by the following examples.

#### Example 1

Sulphate cooking has been performed in autoclaves with a charge of 70 g. bone dry pine chips and with a wood:liquor ratio of 1:4. The alkalinity was 20% and the sulfidity 25%. No addition of black liquor was done. The liquor was added at 70° C. and the temperature increased to 170° C. during 2 hours and kept constant during 2 hours. A varying amount of sodium borohydride (0–2.1% calculated on the wood) was added to the cooking liquor prior to charging. The obtained pulps were washed and screened and yield, Roe number, brightness and strength properties were determined. The beating was performed in a PFI-mill. The following results were obtained.

| Cooking No. | Sodium borohydride (calculated on the wood), percent | Roe number | Yield of unbleached pulp (calculated on the wood), percent | Brightness, percent GE | Beating revolutions | Slowness, °SR | Breaking length, km. | Bursting strength, km./cm. <sup>2</sup> | Tear factor | Double fold |
|-------------|------------------------------------------------------|------------|------------------------------------------------------------|------------------------|---------------------|---------------|----------------------|-----------------------------------------|-------------|-------------|
| 1-----      | 0                                                    | 4.3        | 46.2                                                       | 32                     | 18,000              | 41            | 9.9                  | 8.1                                     | 160         | 6,700       |
| 2-----      | 0.7                                                  | 4.3        | 50.3                                                       | 35                     | 18,000              | 52            | 10.6                 | 8.8                                     | 140         | 11,500      |
| 3-----      | 2.1                                                  | 4.4        | 52.1                                                       | 35                     | 18,000              | 52            | 10.0                 | 8.2                                     | 138         | 8,500       |

such as alkali metal borohydrides and alkali metal aluminium hydrides, e.g. sodium borohydride, potassium borohydride and lithium aluminium hydride. Gaseous hydrogen can also be utilized.

The amount of reducing agent used should suitably be at least 0.001% and preferably at least 0.01% by weight of the lignocellulosic material. Upwardly the amount of reducing agent to be used is limited only by

As is seen from the table an addition of sodium borohydride increases the yield at constant degree of delignification from 46.2% without an addition to 50.3% respectively 52.1% with an addition of 0.7 respectively 2.1% of sodium borohydride corresponding to an increase of 8.9% respectively 12.8%. It can furthermore be seen that an addition of sodium borohydride increases the brightness as well as the beatability of the pulp.

3  
Example 2

Soda cooking was performed in autoclaves with a charge of 70 g. bone dry spruce chips and a wood : liquor ratio of 1:4. The amount of added alkali was 30% sodium hydroxide calculated on the wood. No addition of black liquor was made. The liquor was charged at a temperature of 70° C. and the temperature was increased to 170° C. during 2 hours and was kept constant at that temperature during 2 hours. Varying amount of sodium borohydride (0-2.1% calculated on the wood) was added to the cooking liquor prior to charging. The obtained pulp was washed and screened and yield and Roe number were determined. The following results were obtained.

| Cooking No. | Sodium borohydride (calculated on the wood), percent | Roe number | Yield of unbleached pulp (calculated on the wood), percent |
|-------------|------------------------------------------------------|------------|------------------------------------------------------------|
| 1-----      | 0                                                    | 6.8        | 42.1                                                       |
| 2-----      | 0.7                                                  | 6.2        | 45.9                                                       |
| 3-----      | 2.1                                                  | 6.1        | 47.8                                                       |

As is seen from the table an addition of sodium borohydride increases the yield at constant degree of delignification.

Example 3

Sulphate cooking has been performed in autoclaves with a charge of 70 g. bone dry pine chips and with a wood : liquor ratio of 1:4. The alkalinity was 20% and the sulfidity 25%. No addition of black liquor was done. Prior to charging the chips were impregnated with a liquor being 0.1 N NaOH and containing varying amount of sodium borohydride. All the impregnation liquor was added during an impregnation time of 3½ hours at 20° C. The cooking liquor was added at 70° C. and the temperature increased to 170° C. during 2 hours and kept constant at that temperature during 2 hours. The obtained pulps were washed and screened. Yield and Roe number were determined. The following results were obtained.

| Cooking No. | Sodium borohydride (calculated on the wood), percent | Roe number | Yield of unbleached pulp (calculated on the wood), percent |
|-------------|------------------------------------------------------|------------|------------------------------------------------------------|
| 1-----      | 0                                                    | 4.1        | 45.6                                                       |
| 2-----      | 0.2                                                  | 4.1        | 45.6                                                       |
| 3-----      | 0.4                                                  | 4.0        | 47.0                                                       |
| 4-----      | 0.6                                                  | 3.7        | 48.6                                                       |
| 5-----      | 0.8                                                  | 4.2        | 49.3                                                       |

As is seen from the table an addition of sodium borohydride to the wood in an impregnation stage increases the yield at a constant degree of delignification.

Example 4

Sulphate cooking was performed in autoclaves with continuous liquor flow. The wood charge was 70 g. bone dry pine chips and the cooking liquor had a flow speed of 2 liter/hour. The cooking liquor contains 10 g. sodium hydroxide and 10 g. sodium sulphate per liter. In some cases the wood was pretreated in an impregnation stage

with 0.1 N sodium hydroxide containing 2% sodium borohydride calculated on the wood for 16 hours at 20° C. In some of the experiments the cooking liquor contained an addition to the chemicals needed for delignification also 1 g./l. sodium borohydride. The cooking was started at 70° C. and the temperature increased to 170° C. during 2 hours and were kept constant at that temperature during an additional 2 hours. The obtained pulps were washed and screened. Yield and Roe numbers were determined. The following results were obtained.

| Cooking No. | Impregnation with NaBH <sub>4</sub> | NaBH <sub>4</sub> in the cooking liquor during temperature increase | NaBH <sub>4</sub> in the cooking liquor at 170° C. | Roe number | Yield of unbleached pulp (calculated on the wood), percent |
|-------------|-------------------------------------|---------------------------------------------------------------------|----------------------------------------------------|------------|------------------------------------------------------------|
| 15          |                                     |                                                                     |                                                    |            |                                                            |
| 1-----      |                                     |                                                                     |                                                    | 7.0        | 46.8                                                       |
| 2-----      |                                     |                                                                     |                                                    | 4.0        | 43.7                                                       |
| 3-----      | +                                   |                                                                     |                                                    | 7.0        | 51.5                                                       |
| 4-----      | +                                   |                                                                     |                                                    | 4.0        | 45.5                                                       |
| 5-----      | +                                   | +                                                                   |                                                    | 7.0        | 55.0                                                       |
| 6-----      | +                                   | +                                                                   |                                                    | 4.0        | 51.0                                                       |

As is seen from the table an addition of sodium borohydride to the wood in an impregnation stage results in increased yield at unchanged degree of delignification as far as sulphate cooking is concerned. The increase in yield is, however, greater if sodium borohydride also is added during the temperature increase period of the cook. The increase in yield is approximately 4.5% calculated on the wood when sodium borohydride is present only in the impregnation stage but when sodium borohydride is present during the impregnation stage as well as during temperature increase period of the sulphate cook the increase in yield is approximately 8%, i.e. an additional 3.5%. This is true when the cook is performed to a Roe number of 7 whereas another distribution of the increase in yield is obtained when the cooking is performed to a lower Roe number as is also seen from the table.

I claim:

1. In the preparation of pulp for papermaking by the digestion of wood chips in an alkaline medium at a temperature of between 160° and 200° C., the improvement which comprises carrying out the digestion in the presence of a reducing agent selected from the group consisting of hydrogen and metal borohydrides.
2. The method as set forth in claim 1, in which the reducing agent is added during the temperature increase period of the digestion.
3. The method as set forth in claim 1 in which the reducing agent is an alkali metal borohydride.
4. The method as set forth in claim 1 in which the reducing agent is sodium borohydride.
5. The method as set forth in claim 3 in which the amount of the reducing agent is between 0.01% and 3.00% by weight of the wood chips.

References Cited in the file of this patent

UNITED STATES PATENTS

60 2,898,333 Jullander \_\_\_\_\_ Aug. 4, 1959

OTHER REFERENCES

65 Meller: Studies on Modified Cellulose, TAPPI, volume 38, No. 11, November 1955, pages 682-687.